

Patented Jan. 18, 1927.

1,614,611

# UNITED STATES PATENT OFFICE.

GEBHARDT E. GRIMM, OF SPRINGFIELD, MASSACHUSETTS, ASSIGNOR TO WESTFIELD RIVER PAPER COMPANY, OF RUSSELL, MASSACHUSETTS, A CORPORATION OF MASSACHUSETTS.

## PAPER AND PROCESS OF COATING THE SAME.

No Drawing.

Application filed January 14, 1925. Serial No. 2,441.

This invention is an improvement in paper, and in methods of coating the same, and with respect to its more specific features in metal coated paper.

5 Such papers are used for many purposes, since they are not only highly ornamental, but moisture and germ proof, the base paper being water proofed. For instance, they are used as linings for containers of many types, 10 and ornamental wrappings for packages, of comestibles, such as candies, fruits and the like, and other commodities which it is desired to retain out of contact with the atmosphere.

15 Such paper heretofore has been prepared either by coating a suitable web with a size or varnish, and dusting with the metallic powder, or by coating the paper with an emulsion of the metal. The latter practice 20 is not satisfactory, since it is impracticable to so coat the water proofed or grease proofed paper in ordinary coating machines.

The product of the former practice is not suitable for use with comestibles, or any 25 commodity having a flavor and aroma of its own, such as tobacco products and the like, since the odor of the size or varnish persists after most thorough drying.

The product in the former practice is 30 prone to lack of uniformity in the distribution of the powder, and this may be due to defective work in either stage. The size or varnish may be unequally distributed, in which case there will be a corresponding lack 35 of uniformity in distribution of the powder, or the fault may be due to the unequal spreading of the powder.

In the former instance, the powder lies 40 upon the surface of the varnish, or is but slightly embedded therein, so that the raw surface of the powder is outward. Thus the paper is harsh and unpleasant to the touch lacking the smooth finish desirable in such paper. Moreover the superficial dust 45 particles are easily dislodged when the paper is handled. Such paper is not well adapted for embossing, an operation which is desirable in the most highly finished paper.

In coating with an emulsion of the powder, it is desirable that the paper be water and grease proofed and coated at a single 50 operation, and the vehicles heretofore used for the powder have not been of a character to thoroughly accomplish this purpose,

while at the same time presenting a paper 55 surface satisfactory from all standpoints.

One of the objects of the present invention is the provision of a paper, and a method of coating the same with metallic dust of any selected kind in a single operation. 60

Another object is to provide a vehicle for the metal dust, which not only securely fixes the particles to the paper, but simultaneously moisture and grease proofs the same.

Another object is the provision of a paper 65 uniformly coated, presenting a coating pleasing to the sense of both sight and touch, and inoffensive to the sense of smell.

Another object is the provision of a paper 70 wherein the coating is soft and flexible and the paper is capable of being deeply embossed without marring the coating.

With these and other objects in view the invention consists in the article, and in the process of making the same as defined in the 75 claims appended hereto; it being understood that various changes may be made in the character and the proportions of the ingredients, within the scope of the claims.

The preferred vehicle for the metallic 80 powder, whether applied in emulsion or by powdering includes a fixative and water proofing agent, a softening agent, and a solvent. The vehicle which fixes the powder to the paper whether mixed prior to the 85 time of application or at such time, is a solution of bleached shellac and borax (sodium borate) in water, with an admixture of a waxy material, the amount depending upon the quality of paper desired. 90

In preparing the vehicle 6 to 8 ounces of borax is dissolved in a gallon of water, by bringing the water to a boil after or during the addition of the borax. The shellac 1½ to 2½ pounds is then stirred into the water, 95 which is afterwards permitted to cool.

Either beeswax or paraffin wax may be used. The former may be dissolved in pearl-ash, and the latter is preferably used with stearic acid and japan wax, in about equal proportion. The wax is dissolved in borax water, enough being used to saponify the wax, and to bring to a creamy consistency, very nearly resembling cold cream, the proportions of each being regulated by the results desired. 100

The vehicle prepared as above described, is mixed with the metallic powder in about the

proportions of 40 to 50 pounds of the powder in 15 to 25 gallons of the vehicle.

From 3 to 6 gals. of either of the wax emulsions above mentioned is added to 15 to 25 gals. of the borax and shellac solution, the purpose of the wax being to soften the hard shellac, so that the coating is flexible, soft and velvety to the touch.

The mixture of vehicle and metallic powder is applied to the paper in any suitable manner, usually by means of a coating roller or brush. Since the powder is thoroughly mixed with the vehicle, the parts of each particle being coated thereby, the vehicle 10 completely covers and embeds the particles, and since the vehicle is transparent when dry, the full sheen and lustre of the powder are brought out.

Preferably the paper used is relatively thin and highly calendered, and the peculiar treatment to which it is subjected permits the sheen of the paper to be visible to a certain extent through the coating. This fact may be utilized to provide different color effects, 20 the basic paper being tinted for this purpose.

Because of the quality of the paper forming the subject matter of my co-pending application Ser. No. 2440 of even date herewith, it is especially adapted for use in the 20 present process. The paper in question is coated with a hard resin, (lac or shellac), a softening agent, (soft gum such as elemi or a suitable oil), and a dry wax, all in alcoholic solution. By a dry wax is meant a wax from which the greatest possible amount of water has been removed, as by expression.

Since these ingredients are applied in alcoholic solution and the metallic powder is added directly to the solution, it is obvious 10 that the ingredients are dissolved in the alcohol instead of in water. The principle however is the same, since alcohol can be used as the solvent with the borax and shellac in the formula first mentioned.

Any character of metallic powder may be used in the present process except argentine which requires an adhesive, and the paper may be previously tinted if desired. It may be also embossed or otherwise figured with 15 out lessening the pleasing appearance and attractiveness of the coating. The coating is extremely flexible, and the embossing does not cause any break in the same.

In the present process the powder is coated with the vehicle by means of which it is held to the paper, so that instead of presenting a comparatively rough surface of powder, the paper presents a smooth relatively soft and flexible surface of lacquer or varnish.

The improved paper has a smoothness of

finish far superior to that prepared by old methods, which is in effect sandpaper. The lacquering of the dust that is the mixing of the same with a transparent or semi-transparent varnish or lacquer permits a degree 65 of light reflection from the polished surface of the paper so that the sheen of the paper body is more or less visible as a sheen by reflected light. With the usual method the dry dust makes an opaque shield or screen 70 through which no light can pass, and all of the color is due to light reflection from the dust itself. By suitable coloring of the paper a changeable silk or iridescent effect may be obtained.

As previously stated argentine requires an additional ingredient, namely an adhesive. The brilliancy of argentine paper may however be greatly increased and a better surface obtained by coating the paper with the 80 solution above described.

I claim:

1. Art paper with a semi-transparent burnished body and a coating of metallic powder in a hard flexible transparent fixative including lac, through which the sheen of the body and the powder are visible.

2. Semi-transparent highly calendered art paper, with a coating of metallic powder in a fixative agent of shellac and a waxy substance.

3. Art paper with a semitransparent burnished tinted body, and a coating of metallic powder in a hard transparent fixative including lac, through which coating 95 the sheen of the paper is visible.

4. The process of coating paper, which consists in mixing a metallic powder with a vehicle composed of water shellac, and a waxy substance, and coating the paper with the 100 vehicle.

5. The process of producing art paper, which consists in applying to a semitransparent burnished paper, a coating of a hard flexible transparent fixative including lac 105 and containing a metallic powder, through which coating the sheen of the paper is visible.

6. The process of coating paper, which consists in applying to the paper a metallic 110 powder in a vehicle composed of shellac 15 to 25 pounds, borax 10 to 15 pounds, wax emulsion 3 to 6 gallons, water 15 gallons, and containing 40 to 50 pounds of the metallic powder.

Signed at New York in the county of New York and State of New York this 9th day of January, A. D. 1925.

GERHARDT E. GRIMM.